

# United States Patent

Meyer et al.

[15] 3,668,083

[45] June 6, 1972

[54] **PROCESS OF ELECTROPLATING RHENIUM AND BATH FOR THIS PROCESS**

- [72] Inventors: Andre Meyer, Geneva, Switzerland; Donald Gardner Foulke, Passaic, N.J.
- [73] Assignee: Sel-Rex Corporation, Nutley, N.J.
- [22] Filed: Oct. 27, 1970
- [21] Appl. No.: 84,505

**Related U.S. Application Data**

- [63] Continuation of Ser. No. 739,165, June 24, 1926, abandoned.

[30] **Foreign Application Priority Data**

- July 3, 1967 Switzerland ..... 9470/67
- [52] U.S. Cl. .... 204/43, 204/47
- [51] Int. Cl. .... C23b 5/32, C23b 5/24

[56]

**References Cited**

**UNITED STATES PATENTS**

- 3,260,658 7/1966 Churchward ..... 204/109

**OTHER PUBLICATIONS**

Eldridge K. Camp, Plating, pp. 413-416, May 1965.

*Primary Examiner*—G. L. Kaplan  
*Attorney*—Greene & Durr

[57]

**ABSTRACT**

The invention relates to a bath for electrodepositing low-stress rhenium and its alloys of the perrhenate type and is characterized by the addition of ions which make up one or more of the following salts: magnesium sulfate, magnesium sulfamate, aluminum sulfate and aluminum sulfamate. The invention also relates to the process of electroplating from said bath.

**10 Claims, No Drawings**

## PROCESS OF ELECTROPLATING RHENIUM AND BATH FOR THIS PROCESS

This application is a continuation of our U.S. Pat. application, Ser. No. 739,165, filed June 24, 1968 and now abandoned.

The present invention relates to a method for the electrodeposition of rhenium and to a bath for carrying out this method.

Rhenium has many interesting properties. Its melting point is 3,180° C., its oxide is conductive and this metal is very hard and has a high density as well as good reflectivity. These properties suggest its use under suitable high temperature conditions, for switching devices, as a protecting material against radiations and as a thermal shield.

Rhenium has been plated for more than thirty years. However, the baths described in the literature give in general brittle deposits, many cannot be used for heavy deposits and have efficiencies of under 10 percent.

Many formulations for rhenium plating baths have been disclosed in the literature, all of which comprise the use of solutions containing perrhenate ions,  $\text{ReO}_4^-$ .

The object of the present invention is to provide a method and an electrolytic bath for the deposition of rhenium to heavy thicknesses at a good efficiency. A second object of the invention is to permit the deposition of the rhenium in a low-stressed ductile condition.

The method, according to the invention, is characterized by the fact that one uses a bath containing rhenium as the perrhenate ion and a salt selected from the group comprising magnesium sulfate, magnesium sulfamate, aluminum sulfate and aluminum sulfamate.

The bath according to the invention is characterized by the fact that it contains rhenium as the perrhenate ion and a salt selected from the group comprising magnesium sulfate, magnesium sulfamate, aluminum sulfate and aluminum sulfamate.

It has been ascertained that the addition of magnesium sulfate and magnesium sulfamate to a bath containing the perrhenate ion adjusted to a pH value of less than 10 will produce thick, low-stressed deposits. Furthermore, the bath efficiency, although still rather low, is of the order of 12 to 13 percent of the theoretical. When the pH is raised above 2, the efficiency begins to fall off, so that a pH range of 1 to 2 is preferable. The pH may be reduced with sulfuric or a phosphoric acid. Hydrochloric acid is not advisable because chlorides are detrimental. It is the magnesium ion which is effective but, obviously, magnesium oxide and carbonate can be added because they will be converted to sulfate or sulfamate in the solution.

The deposits are adherent, smooth and fully bright. Satisfactory deposits have been obtained on many basis metals. Where the high acidity attacks the basis metal, it should be plated first with nickel. In order to prevent contamination of the bath, the use of a gold strike, prior to the rhenium plating step, has been found helpful.

A typical bath, in grams per liter, is the following:

|                                                          |                             |
|----------------------------------------------------------|-----------------------------|
| Potassium Perrhenate (K $\text{ReO}_4$ )                 | 10 g/l                      |
| Sulfuric acid (H $_2$ SO $_4$ )                          | 30 ml/l                     |
| Magnesium sulfate (MgSO $_4 \cdot 7\text{H}_2\text{O}$ ) | 25 g/l                      |
| CONDITIONS:                                              |                             |
| pH:                                                      | 1.0                         |
| Current density:                                         | 10 Amp/dm $^2$<br>(2 to 30) |
| Temperature: 60° (20 to 95°C)                            |                             |

### EXAMPLE 1

Deposits were obtained from this bath which were bright and hard, at an efficiency of 11.2 percent. At a current density of 20 Amp/dm $^2$ , the efficiency was 12.4 percent; at 15 Amp/dm $^2$ , the efficiency was 11.9 percent, at 25° C. and at 10 Amp/dm $^2$  the efficiency was 10.1 percent when the pH was raised to 10.0, the efficiency was 9.2 percent.

The temperature of the bath can be varied from 20° to 95° C. but a temperature of 60° C. appears to be most satisfactory

in that the efficiency is good and the evaporation of the solution is not excessive.

### EXAMPLE 2

5 The substitution of 25 g/l of magnesium sulfamate for the magnesium sulfate in the typical bath described above yielded deposits which appear to be even less stressed on the basis of a qualitative test, so it appears that the magnesium ion is the effective agent, but that the anion also has an effect. The deposits were bright and adherent to the nickel basis metal provided with a gold-strike. The amount of rhenium added as the perrhenate ion is not limited to 10 g/l as given in the example. This may be varied from 2 g/l to 50 g/l. For cost reasons, 10 the concentration of rhenium is usually from 10 to 15 g/l.

15 The amount of magnesium salt required is not critical in that it can be varied over a wide range. However, it appears that the lower limit at which the salt is effective is about 5 g/l and that quantities above 50 g/l do not produce any improvement. 20 However, the scope of the invention is not limited to the higher value mentioned, because amounts of magnesium salt up to saturation can be used.

25 It is possible to add metallic ions to the magnesium-containing perrhenate solution and to obtain alloys which, likewise, exhibit low stress. Nickel, cobalt, indium and gold have been codeposited with rhenium.

### EXAMPLE 3

30 Examples 1 and 2 indicate the simplest formulation, i.e., a solution containing the perrhenate ion and magnesium sulfate with the pH lowered to 1 or 2 with sulfuric and sulfamic acids respectively. The amount of acid is conveniently 2 to 25 g/l, but these data are not critical. It is sometimes helpful to add to 35 the simple solutions conducting salts such as ammonium sulfate or sulfamate. A typical formula is as follows:

|                      |                |
|----------------------|----------------|
| Potassium perrhenate | 10 g/l         |
| Sulfuric acid        | 10 g/l         |
| Ammonium sulfate     | 25 g/l         |
| Magnesium sulfate    | 25 g/l         |
| CONDITIONS:          |                |
| pH:                  | 2              |
| Current density:     | 12 Amp/dm $^2$ |
| Temperature:         | 65°C           |

Deposits obtained from this bath were bright and hard and the current density efficiency was 10 percent.

### EXAMPLE 4

50 A typical alloy bath is as follows:

|                                            |                |
|--------------------------------------------|----------------|
| Ammonium perrhenate (NH $_4\text{ReO}_4$ ) | 10 g/l         |
| Sulfuric acid                              | 30 ml/l        |
| Ammonium sulfate                           | 25 g/l         |
| Magnesium sulfamate                        | 25 g/l         |
| Nickel sulfate                             | 20 g/l         |
| CONDITIONS:                                |                |
| pH:                                        | 1              |
| Current density:                           | 12 Amp/dm $^2$ |
| Temperature:                               | 60°C           |

60 It has been moreover discovered that a bath containing the perrhenate ion along with magnesium sulfate and/or sulfamate along with the perchlorate ion will produce thick, low-stressed deposits at a plating rate of almost 3 mg/Ampere-minute. 65 These baths are more efficient at a pH of 1 to 2 but are operable at higher pH and at a slower rate of deposition.

66 It has also been ascertained that the corresponding aluminum salts may be substituted for the magnesium sulfate and for the magnesium sulfamate. 70 The deposits are adherent, smooth and brighter than these previously obtained. Since the bath is normally quite acid, it is advisable to preplate acid-soluble basis metals with nickel, the nickel coating itself should be goldflashed to minimize the contamination of the bath by nickel impurities. Of course, when plating rhenium-nickel alloys, this is not necessary.

## EXAMPLE 5

A bath was prepared containing:

|                                            |         |
|--------------------------------------------|---------|
| Rhenium (as potassium perrhenate)          | 6 g/l   |
| Magnesium sulfate ( $MgSO_4 \cdot 7H_2O$ ) | 40 g/l  |
| Sulfuric acid                              | 30 ml/l |
| Sulfamic acid                              | 40 g/l  |
| Sodium perchlorate                         | 10 g/l  |

Deposits obtained from the above bath at 60° C. and at 10 Amp/dm<sup>2</sup> were bright and ductile. The plating rate was 2.78 mg/Ampere-minute while the rate for the standard bath, containing neither the perchlorate nor the magnesium sulfate, is of the 1.2 mg/Ampere-minute. Adding the magnesium sulfate only, but not the perchlorate as in Example 3, increased the rate of 1.5 mg/Ampere-minute. The addition of the perchlorate improved this rate by more than 80 percent, bringing it to the above mentioned figure of 2.78 mg/Ampere-minute, the depositing having moreover a brighter appearance.

## EXAMPLE 6

A bath was prepared containing:

|                         |         |
|-------------------------|---------|
| Rhenium (as perrhenate) | 6 g/l   |
| Aluminum perchlorate    | 10 g/l  |
| Sulfamic acid           | 30 g/l  |
| Magnesium sulfate       | 40 g/l  |
| Sulfuric acid           | 30 ml/l |

At 10 Amp/dm<sup>2</sup> and 60° C. bright deposits were obtained from this bath, at the rate of 2.47 mg/Ampere-minute.

## EXAMPLE 7

To the bath described in Example 5 were added 20 g/l of nickel sulfate. The deposit was bright and rather ductile, differing in color from that of Example 5, indicating the formation of a rhenium-nickel alloy. The plating conditions were the same as for Example 5.

## EXAMPLE 8

To the bath of Example 6 were added 10 g/l of cobalt sulfate and, as in this example, a bright alloy deposit was obtained.

The features and principles underlying the invention described above in connection with specific exemplifications will suggest to those skilled in the art many other modifica-

tions thereof. It is accordingly desired that the appended claims shall not be limited to any specific feature or details thereof.

We claim:

- 5 1. An aqueous electroplating bath for the electrodeposition of low-stress deposits of rhenium and its alloys comprising from 2 to 50 grams of rhenium as the perrhenate ion per liter of bath, and the ions from at least one salt selected from the group consisting of magnesium sulfamate, aluminum sulfate, and aluminum sulfamate, the concentration of said salt ranging from about 5 grams per liter of bath up to its saturation concentration, said bath being maintained at a pH of less than 10.
- 10 2. The aqueous electroplating bath of claim 1 comprising in addition at least one conducting salt selected from the group consisting of alkali metal and ammonium salts of sulfuric, sulfamic and perchloric acids.
- 15 3. The aqueous electroplating bath of claim 1 comprising in addition free acid selected from the group consisting of perchloric, sulfuric and sulfamic acids.
- 20 4. The aqueous electroplating bath of claim 1 comprising, in addition to the perrhenate ions, ions of an electrodepositable metal, added as a soluble salt of the metal.
- 25 5. The aqueous electroplating bath of claim 1 wherein the bath is maintained at a pH of 1 to 2.
- 25 6. A method of electrodepositing rhenium and its alloys which comprises electrolyzing, at a current density of 2 to 30 amp/dm<sup>2</sup> measured at the cathode, an aqueous bath comprising from 2 to 50 grams of rhenium as the perrhenate ion per liter of bath and at least one salt selected from the group consisting of magnesium sulfate, magnesium sulfamate, aluminum sulfate and aluminum sulfamate, the concentration of said salt ranging from about 5 grams per liter of bath up to its saturation concentration, said bath being maintained at a pH of less than 10.
- 30 7. The method of claim 6 wherein said bath contains at least one conducting salt selected from the group consisting of alkali metal and ammonium salts of sulfuric, sulfamic and perchloric acids.
- 35 8. The method of claim 6 wherein said bath contains in addition free acid selected from the group consisting of perchloric, sulfuric and sulfamic acids.
- 40 9. The method as claimed in claim 6 wherein said bath contains, in addition to the perrhenate ion, at least one ion of a metal which is codeposited with the rhenium.
- 45 10. The method of claim 6 wherein the bath is maintained at a pH of 1 to 2.

\* \* \* \* \*